

Oct. 7, 1958

P. DELRIEU

2,855,264

ACTIVATED ELECTRODE FOR ELECTRIC DISCHARGE LAMP

Filed Sept. 20, 1955



INVENTOR

PIERRE DELRIEU  
By Young, Frenay & Thompson  
ATTYS.

2,855,264

## ACTIVATED ELECTRODE FOR ELECTRIC DISCHARGE LAMP

Pierre Delrieu, Paris, France, assignor to Societe Anonyme pour les Applications de l'Electricite et des Gaz Rares-Etablissements Claude-Paz & Silva, Paris, France

Application September 20, 1955, Serial No. 535,331

Claims priority, application France September 22, 1954

2 Claims. (Cl. 316—8)

This invention relates to processes for manufacturing electric discharge lamps which contain an ionizable discharge atmosphere and which have at least one activated electrode, and more particularly to those lamps in which the discharge atmosphere has an absolute pressure higher than 0.5 kg./cm.<sup>2</sup> during the operation of the lamp, the envelope of which is made of a vitreous material having a very high silica content and the activated electrode, or electrodes, of which comprise a refractory metal member provided with electron-emissive material, said electron-emissive material being obtained from a substance which has a melting point higher than 2500° C. and which produces, during the formation of the electrode, only products among which those which are not gaseous in the conditions of their production have melting points higher than 2500° C., these melting points being measured in the conditions to which the substance and products are subjected when the lamp is being manufactured.

In the above definition of the substance, the term "formation of the electrodes" does not comprise the electric discharges to which electrodes are sometimes subjected before the lamp is put into normal service, for instance so as to convert a small fraction of the alkaline-earth oxides which activate them into alkaline-earth metal.

The conditions to which the substance and products are subjected when the lamp is being manufactured and which may influence the melting points thereof are, for example, the pressures to which the substance and products are subjected.

The products originating from said substance may be temporary products, that is products which will be transformed during later formation operations on the electrode, as well as permanent products, which will not be transformed any further.

In the known processes for manufacturing discharge lamps the envelope of which has a very high silica content, the activated electrodes are heated by various methods for their formation but all these processes are relatively difficult to realize. For instance, heating an electrode by flowing an electric current through the member which supports the electron-emissive material necessitates two lead wires for the electrode, but the manufacture of lead wires is difficult when they must be sealed vacuum-tight in a vitreous material having a very high silica content. Heating the support member by discharges or by induced eddy currents is also difficult, the induction, for example, requiring magnetic fields difficult to obtain in the case of electrodes the diameter of which is small and which do not comprise ferromagnetic metal.

It is among the objects of the invention to provide a process for manufacturing a lamp of the type above described, which process is easy to use and results more regularly than the known processes in satisfactory lamps.

In accordance with the invention, the substance from which is obtained the electron-emissive material is deposited on the support member for the emissive material in a condition of suspension in a liquid, and the degassing

2

of the lamp and the formation of the activated electrode, or electrodes, of the lamp is effected by heating the whole of the lamp to a temperature higher than 900° C. while pumping the non-inert gases out of the lamp, said electrode, or electrodes, being at that moment located in the lamp.

The pumping of the non-inert gases contained in the lamp may be effected by exhausting the lamp, or by flowing an inert gas through it, or by both these means.

10 Heating the lamp envelope above 1300° C. is generally to be avoided since vitreous silica devitrifies at that temperature.

In the process of the invention the electrode is heated only through the lamp envelope. There is then no need 15 for heating the electrode by another method, more difficult to put into practice, or even impossible which is the case of the flowing of a direct or low frequency electric current when the electrode is provided with one lead-in wire only. This process is easy to use; the envelope may 20 be heated by a gas oven or an electric oven, or by one or more burners, or banks of burners, using gaseous or liquid fuel.

For a better understanding of the invention and to show 25 how the same may be carried into effect, electrodes for 30 which the process of the invention is used, as well as a lamp comprising such electrodes, are represented in the accompanying drawings, in which:

Fig. 1 represents diagrammatically, partly in section, 35 partly in elevation, an electrode fastened to its lead-in wire.

Figure 2 represents diagrammatically, in elevational view, a mercury vapor discharge lamp incorporating two electrodes of the kind shown in Figure 1, the lamp being 40 illustrated during manufacture at a point when these electrodes have just been introduced in the lamp envelope.

Figures 3, 4, 5 represent diagrammatically, in section, other forms of electrode.

In the electrodes shown in Figure 1, the metal part 40 carrying the emissive material comprising a tungsten rod or pin 2, of 1.5 mm. in diameter, and a helix 1 of tungsten wire of 0.5 mm. in diameter through which the rod 2 has been passed. The helix 1 comprises 18 turns of which only ten have been shown for greater clearness of the drawing. The right hand end of the helix is welded electrically to the rod 2. The spacing between two adjacent turns of the helix 1 is, on the average, about 0.05 mm., the clearance between the rod 2 and the helix being of the same order. The composite part 1, 2 has undergone 45 treatments intended to purify the tungsten surface, well known treatments which involve, in particular, successive heatings to about 1000° C. in dry hydrogen and thereafter in wet hydrogen.

Before applying to the composite part 1, 2 a substance 50 which will be transformed into an emissive material, such part is welded, a few millimeters from the left hand end of the helix, to the end of a thin molybdenum strip 4 at the other end of which a thicker strip 17, for example also of molybdenum, is welded to form a lead-in connection to the electrode. The thin strip 4, which is 0.015 mm. thick, except at its edges, which are thinned, is a few centimeters long. It is the sealing of the strip 4 to the quartz of the envelope of the discharge device which will ensure the vacuum tightness of current lead-in 55 connection.

The assembly consisting of the part 1, 2, the thin strip 4 and the lead-in connection 17 is cleaned, for instance, by heating in hydrogen.

The part 1, 2 is then coated, for instance by dipping 60 or by means of a brush, with some calcium carbonate suspension, this coating being carried out in such a way as to fill, by capillarity, the clearances between the turns

of the helix 1 and between said helix and the rod 2. The suspension is then allowed to dry in air, which yields a coat 3 of calcium carbonate. In some cases, the portion of the coat 3 which is on the outer surface of the part 1, 2 is removed with a brush, so as to avoid fouling the envelope of the lamp when its electrodes are introduced therein, if the electrodes then rub the envelope.

The suspension is obtained, for instance, by crushing in a ball mill, for 60 hours, 100 grams of pure calcium carbonate, precipitated, with 100 grams of purified butyl acetate. After this crushing, about 250 grams of butyl acetate are added. With this dilution, the coatings 3 obtained are sufficiently adhesive although they contain no binder, and they contain enough calcium carbonate.

Two semi-finished electrodes 6, 12 thus obtained are introduced into an envelope for a discharge lamp, made of quartz and comprising as represented in Figure 2, a central portion 5 provided with an exhaust tube 11 and two end pieces 8 and 16 which are open to allow the introduction of the electrodes therethrough. One electrode 6, is attached to molybdenum strips 10 and 9, and the other electrode 12, is attached to molybdenum strips 14 and 15. Following the introduction of the electrodes the two end parts are sealed by heating whereafter a vacuum is made through the exhaust tube 11, and the strips 10 and 14 are sealed to the end pieces 8, 16.

Once these two sealing operations are completed the lamp is connected through its exhaust tube 11 with a vacuum pump, and then placed in an oven which raises its temperature to about 1100° C. This treatment, the duration of which is of the order of 15 minutes, results in a removal of gases from the electrode, and in a transformation of calcium carbonate into calcium oxide in accordance with the equilibrium reaction:



This reaction is complete in the direction which produces carbon dioxide, since it is carried out in a vacuum and for a sufficient time.

Once the electrodes have been so treated, there are introduced into the lamp, through the exhaust tube 11, argon and liquid mercury, whereafter the exhaust tube is closed by heating in the vicinity of the tube 5 in a known manner.

During these operations, neither the calcium carbonate nor its decomposition product, calcium oxide have melted. The pressure of the carbon dioxide in contact with coating 3 has always been very far from the high pressures at which it is possible to melt calcium carbonate or even the eutectic thereof with calcium oxide. The temperature reached during the heating in the oven is also very far from the melting point of calcium oxide (about 2580° C.). Since there has been no melting, neither the carbonate nor the calcium oxide have moved and have fouled the envelope of the lamp and formed excess thicknesses of emissive material at the expense of certain portions of the helix 1. The emissive layer is thus very uniform and electrodes manufactured in the same manner will have very similar characteristics.

High intensity discharges often used during the degassing and the forming of the electrodes are unnecessary with the above described process.

Another advantage is that it is possible to manufacture a lamp without any glass sealing after introduction of the electrodes, other than the closing of the exhaust tube and of the two end pieces.

The electrode for which the above numerical data is given is suitable, for example, for mercury vapor lamps operating with a vapor pressure of the order of two atmospheres, a current of several amperes, for instance 3.5 amperes, and a voltage gradient of 5 to 40 volts per centimeter length between electrodes when the inner diameter of the tube 5 is 25 millimeters.

Figure 3 shows, in section, an electrode, in which the metal coil forms two layers. The use of such an electrode, which is shorter than that represented in Figure 1, allows a better heating of the ends of the lamp during the functioning thereof. The coil 19, for example, comprises 15 turns. The outer diameter of the outer layer of the coil should be sufficiently small to allow the electrode to pass through the end piece 8 or 16.

Figure 4 shows an electrode, the coil of which, made of tungsten wire 0.5 mm. in diameter with spacings of 0.05 mm., is divided into two portions: a front portion 20 which is not provided with electron-emitting material, and a rear portion 21, which supports an emissive coat. The portion 20 for instance, may comprise 14 turns and the portion 21 four turns, the distance between the portions 20 and 21 being about 2 millimeters. As indicated, the portion 21 only may be coated by dipping or by using a brush, with the substance which will be transformed into emissive material.

Figure 5 represents an electrode, the coil of which is divided into a front portion 22 with no electron-emissive material, and a rear portion 23 with a coil forming a double layer and having emissive material. The portion 22 may, for example, comprise six turns, and the portion 23 seven turns.

Regarding the activating substance suspension, it is also possible to use a suspension of calcium oxide, obtained, for example, by milling 100 grams of lime in 100 grams of butyl acetate for 6 to 50 hours, then diluting the mixture obtained in 500 grams of butyl acetate. Thorium oxide may also be used. The heating by the oven, through the envelope, may then, in some cases, not be quite so strong as when calcium carbonate is used.

The suspension of activating material may also contain a refractory metal, tungsten for instance, in very finely powdered form, or silica, which may increase the adherence of the emissive material. A binder may also be added, for instance 1% in weight of nitrocellulose with respect to the activating substance.

Metal parts of the electrode may be made of molybdenum or tantalum, instead of tungsten. The coating with the substance which will produce the emissive material may be effected before welding the rod 2 to the thin molybdenum strip 4 of the lead-in.

Still other forms of electrodes may be used.

The discharge atmosphere may be krypton or xenon, with a pressure higher than 0.5 kg./cm.<sup>2</sup> during operating.

What I claim is:

1. In a process for manufacturing an electric discharge lamp containing an ionizable discharge atmosphere and having at least one activated electrode, the discharge atmosphere having an absolute pressure higher than 0.5 kg./cm.<sup>2</sup> during the operation of the lamp, the envelope of the lamp being made of a vitreous material having a very high silica content and said activated electrode comprising a refractory metal member provided with electron-emissive material, said electron-emissive material being obtained from a substance which has a melting point higher than 2500° C. and which produces, during the formation of the electrode, only products among which those which are not gaseous in the conditions of their production have melting points higher than 2500° C., these melting points being measured in the conditions to which the substance and products are subjected when the lamp is being manufactured, the steps of depositing said substance on said refractory metal member in a condition of suspension in a liquid, and of degassing the lamp and forming the activated electrode solely by heating the whole of the lamp to a temperature higher than 900° C. while pumping non-inert gases out of the lamp, said electrode being at that moment located in the lamp and the temperature reached by the envelope during this heating step being at least as high as the temperature reached by the electrode.

2. In the process according to claim 1, the step of depositing on the refractory metal member the substance from which the electron-emissive material is obtained, in a condition of very fine suspension in a slightly volatile liquid.

References Cited in the file of this patent

UNITED STATES PATENTS

5 2,007,926 Braselton \_\_\_\_\_ July 9, 1935  
2,249,672 Spanner \_\_\_\_\_ July 15, 1941